



US007470495B2

(12) **United States Patent**  
**Ono et al.**

(10) **Patent No.:** **US 7,470,495 B2**  
(45) **Date of Patent:** **Dec. 30, 2008**

(54) **ELECTROPHOTOGRAPHIC TONER AND IMAGE FORMING METHOD**

(75) Inventors: **Kaori Ono**, Hino (JP); **Satoru Ikesu**, Fuchu (JP); **Koji Daifuku**, Hachioji (JP)

(73) Assignee: **Konica Minolta Holdings, Inc.** (JP)

(\*) Notice: Subject to any disclaimer, the term of this patent is extended or adjusted under 35 U.S.C. 154(b) by 439 days.

(21) Appl. No.: **11/240,967**

(22) Filed: **Sep. 30, 2005**

(65) **Prior Publication Data**

US 2006/0093935 A1 May 4, 2006

(30) **Foreign Application Priority Data**

Oct. 8, 2004 (JP) ..... 2004-296024

(51) **Int. Cl.**

**G03G 9/08** (2006.01)

(52) **U.S. Cl.** ..... **430/108.1**; 430/110.1; 430/108.4

(58) **Field of Classification Search** ..... 430/108.1, 430/110.1, 108.4

See application file for complete search history.

(56) **References Cited**

U.S. PATENT DOCUMENTS

6,268,103 B1 \* 7/2001 Hopper et al. ..... 430/137.14

2002/0039699 A1 \* 4/2002 Nishimori et al. ..... 430/137.11  
2003/0049559 A1 \* 3/2003 Shigemori et al. ..... 430/137.18  
2003/0138714 A1 \* 7/2003 Hayashi et al. ..... 430/108.3  
2004/0013961 A1 \* 1/2004 Niwa et al. ..... 430/107.1  
2005/0048393 A1 \* 3/2005 Ota ..... 430/137.15  
2005/0064314 A1 \* 3/2005 Fujino et al. ..... 430/110.2  
2005/0100809 A1 \* 5/2005 Fujino et al. ..... 430/110.2  
2005/0136354 A1 \* 6/2005 Ueda et al. ..... 430/110.2

FOREIGN PATENT DOCUMENTS

JP 2-166467 \* 6/1990

OTHER PUBLICATIONS

English language Abstract of JP 02166467 A. Jun. 27, 1990.\*

\* cited by examiner

Primary Examiner—Hoa V Le

(74) Attorney, Agent, or Firm—Squire, Sanders & Dempsey L.L.P.

(57) **ABSTRACT**

An electrophotographic toner exhibiting superior color reproducibility and transparency and improved characteristics is disclosed, comprising a thermoplastic resin and colored microparticles dispersed in the thermoplastic resin and containing a dye and a resin differing in composition from the thermoplastic resin. An image forming method by use of the toner is also disclosed.

**7 Claims, 1 Drawing Sheet**



FIG. 1



FIG. 2



1

## ELECTROPHOTOGRAPHIC TONER AND IMAGE FORMING METHOD

This application claims priority from Japanese Patent Application No. JP2004-296024, filed on Oct. 8, 2004, which is incorporated hereinto by reference.

### FIELD OF THE INVENTION

The present invention relates to a toner for use in electro-photography and an image forming method by use thereof.

### BACKGROUND OF THE INVENTION

Recently, color-copying methods have come into practical use, in which an electrostatic latent image carrier is exposed to spectrally separated light to form an electrostatic latent image of an original and the latent image is further developed with color toners to obtain a colored copy image or the respective color copy images are superimposed to obtain a full color copy image. As toner used in the foregoing are manufactured color toners of yellow, magenta, cyan and the like which are formed by dispersing a dye and/or pigment of the respective colors in a binder resin.

The foregoing electrophotographic process, in general, forms images in accordance with the following steps. First, exposing light information in response to image information onto an electrostatic latent image carrier (hereinafter, also denoted as a photoreceptor) composed of a photoconductive material, through various methods forms a latent image on the photoreceptor. The electrostatic latent image formed on the photoreceptor is developed with a charged toner to form a toner image. The formed toner image is transferred onto an image recording medium (hereinafter, also denoted as transfer material) and fixed onto the transfer material using a thermal fixing apparatus.

In the foregoing color image forming method employing the electrophotographic process, electrostatic latent images formed on the photoreceptor correspond to image information which have been separated to the respective colors of yellow, magenta, cyan and black and developed with a toner having a color identical to the respective image information. The development step is repeated four times for the respective colors to form a full color image.

Organic pigments and dyes known in the art have conventionally been used as a colorant used for electrophotographic toner but they exhibit various defects. For instance, organic pigments are generally superior in heat resistance or lightfastness, compared to dyes but existing in toner particles in the form of granular dispersion results in enhanced masking, leading to reduced transparency. In general, low dispersibility of pigments results in deteriorated transparency and lowered chromaticness, deteriorating color reproducibility of images.

When different color toners are superimposed, transparency of fixed toners is needed to visually confirm color of a toner existing in the lowest layer. Dispersibility or coloring power of a colorant become necessary to maintain color reproducibility of an original.

To overcome the foregoing defects of pigments, there were proposed a technique for enhancing transparency in which application of a flushing process as a means for dispersing pigments achieved a pigment dispersion diameter in the order of sub-microns, formed of primary particles without forming aggregated secondary particles; and a technique for improving electrification property, fixability and image uniformity by covering pigment particles with a binding resin or a shell-resin, as described, for example, in JP-A Nos. 9-26673

2

and 11-160914 (hereinafter, the term, JP-A refers to Japanese Patent Application Publication).

However, even when forming toner images by using the thus proposed toner, it is difficult to achieve sufficient transparency, specifically in the case of a pigment toner.

In color imaging apparatuses, all of color reproduction can be achieved, in principle, by a subtractive color system using the three primary colors of yellow, magenta and cyan. In practice, however, the spectral property provided when dispersing a pigment in thermo-plastic resin or the color-mixing characteristic provided when superimposing different toners results in a reduced range of color reproducibility or lowered chromaticness so that problems to be overcome still remain to achieve faithful color reproduction of an original.

There were also introduced toners using dyes and toners using a mixture of a dye and a pigment. In a toner using a dye, the dye existed in the form of being dissolved in a binding binder so that superior transparency and chromaticness were achieved but inferior lightfastness or heat resistance resulted as compared to pigments, as described, for example, in JP-A Nos. 5-11504 and 5-34980.

With respect to heat resistance, in addition to lowered density due to decomposition of a dye, there were produced problems that when fixing a toner image by a heated roller, the dye was sublimed, easily causing in-machine staining and it was also dissolved in silicone oil used in the fixing stage and finally adhered to the heated roller, causing the so-called off-set phenomenon. To overcome such defects of dyes, there were proposed a technique of using specific anthraquinone type dyes as a magenta toner to improve lightfastness and sublimation ability in compatible with color reproduction and an encapsulated toner in which a core containing polymer resin and a color dye was covered with a polymer, as described, for example, in JP-A Nos. 5-72792 and 8-69128.

However, even when forming toner images using electrophotographic toners, as proposed above, it was difficult to achieve sufficient heat resistance (sublimation resistance) and lightfastness.

### SUMMARY OF THE INVENTION

The present invention has come into being as a result of the extensive study to overcome the foregoing problems. It is an object of the present invention to provide a toner for electrophotography enabling superior coloring without producing any problems in dispersion in thermo-plastic resin and exhibiting superior color reproducibility and transparency and improved charging property, off-set resistance and heat resistance.

Thus, in one aspect the present invention is directed to an electrophotographic toner comprising a thermoplastic resin and colored microparticles dispersed in the thermoplastic resin and containing a dye and a resin differing in composition from the thermoplastic resin.

In another aspect the invention is directed to an image forming method comprising developing an electrostatic latent image formed on a support for the electrostatic image with a toner to form a toner image, and transferring the formed toner image to a transfer material, wherein the toner is the electrophotographic toner, as described above.

### BRIEF EXPLANATION OF THE DRAWING

FIG. 1 illustrates the section of a toner particle containing colored microparticles dispersed in thermoplastic resin.

FIG. 2 illustrates the section of a colored microparticle having a core/shell structure, formed of a core covered with a shell resin.

#### DETAILED DESCRIPTION OF THE INVENTION

In one aspect of this invention, the toner for electrophotography (hereinafter, also denoted simply as a toner) comprises a thermoplastic resin and colored microparticles dispersed in the thermoplastic resin, and the colored microparticles contain a resin having a composition different from the thermoplastic resin and a dye. Thus, instead of dispersing or dissolving a dye in a binding resin used for a toner generally known as a toner using a dye, colored microparticles which contain a resin differing in composition from the foregoing thermoplastic resin and a dye, are dispersed in the thermoplastic resin.

A dye of the colored microparticles is dissolved in the resin at the molecular level, enabling elimination of a component such as covering particles to shield light, whereby enhanced transparency of a single-color toner results and transparency of superposed colors is also enhanced.

Constitution of the toner of this invention will now be described with reference to illustrations.

FIG. 1 is a sectional view of a toner particle (1) comprised of colored microparticles dispersed in thermo-plastic resin. In FIG. 1, numeral 1 designates a toner particle, numeral 2 is thermoplastic resin, numeral 3 is a colored microparticle, numeral 4 is a resin and numeral 5 designates a dye. As apparent from FIG. 1, the toner particle is composed of a thermoplastic resin in which colored microparticles are dispersed, and the microparticles are each composed of a resin and a dye.

As shown in FIG. 2, the toner particle may be a particular resin composed of a particular interior (core) containing resin and a dye, and further thereon, covered with a shell resin (or denoted simply as a shell). In that case, the combination of a resin forming the interior (core) of colored microparticles with a thermoplastic resin (binding resin) is not specifically limited, the degree of freedom is broad with respect to material. If only a shell resin (core) is identical with respect to four colors of the toner (yellow, magenta, cyan, black), manufacturing is performed under similar conditions, leading to enhanced advantage in cost. Migration of a colorant dye to the outside of the particular resin (bleeding-out onto the surface of the colored microparticle) does not occur so that there is no fear of sublimation of a dye or oil staining during fixing which is often caused in conventional dye toners.

FIG. 2 illustrates the section of a colored microparticle (3) having a core/shell structure, formed of a core covered with a shell resin. In FIG. 2, numeral 6 designates the interior (core) and numeral 7 designates the exterior resin (or shell), in which the interior (core) is a microparticle containing a resin and a dye.

Preparation of colored microparticles relating to this invention will now be described.

The colored microparticles can be obtained by dissolving (or dispersing) a resin and a dye in an organic solvent and emulsifying them in water, followed by removal of the organic solvent. When covering with a shell resin (shell), a polymerizable monomer containing an unsaturated double bond is added thereto and emulsion polymerization is performed in the presence of a surfactant. Thus, concurrently with polymerization, deposition onto the core surface is performed to obtain colored microparticles having a core/shell structure. The colored microparticles can be obtained by various methods. For example, an aqueous dispersion of resin

microparticles is formed in advance through emulsion polymerization, then, an organic solvent solution containing a dye is added to the aqueous dispersion of resin microparticles to allow the dye to be impregnated in the resin microparticles to form colored microparticles. Then, a shell is formed on the colored microparticles as a core.

The shell is formed preferably of an organic resin. Shell formation (or shelling) can be performed by dropwise adding a resin dissolved in an organic solvent to allow deposited resin to adsorb onto the colored microparticle surface. In the preferred method of shell formation, colored microparticles as a core are formed, then, a polymerizable unsaturated monomer containing a double bond is added thereto in the presence of a surfactant to perform emulsion polymerization and the formed polymer is deposited on the core surface, forming a shell.

In this invention, the core/shell structure means a form in which at least two resins or dyes differing in composition exist, while being phase-separated from each other. In addition to the form of a shell completely covering the core portion, the shell may only partially cover the core. A part of a resin forming the shell may form a domain within the core. Further, it may be a multi-layer structure of at least three layers including at one layer between the core portion and the shell portion.

In this invention, colored microparticles each form a core/shell structure. A core/shell structure having a colored portion formed of a resin and a dye of the colored microparticles, as a core, which is further covered with an exterior resin to form a shell.

Thermoplastic resin contained in the toner of this invention is preferably one which exhibits high adhesion to the colored microparticles, and a solvent-soluble thermoplastic resin is specifically preferred. When a precursor of a thermoplastic resin is solvent-soluble, a curable resin forming a three-dimensional structure is also usable.

Thermoplastic resins which are conventionally used as a binding resin for toners, are usable. Preferred examples thereof include acryl resin such as styrene resin, alkyl acrylate and alkyl methacrylate, styrene acryl copolymer resin, polyester resin, silicone resin, olefin resin, amide resin and epoxy resin. There is desired a resin exhibiting enhanced transparency and melt characteristics such as low viscosity and sharp-melting property to enhance transparency or color reproduction of superposed images. Styrene resin, acryl resin and polyester resin are suitable as a binding resin having such characteristics.

Thermoplastic resins having the following characteristics are preferred. Thus, the number-average molecular weight (Mn) is preferably from 3000 to 6000, and more preferably from 3500 to 5500. The ratio of the weight-average molecular weight (Mw) to the number-average molecular weight (Mn), that is Mw/Mn, is preferably from 2 to 6, and more preferably 2.5 to 5.5. The glass transition temperature is preferably from 50 to 70° C. and more preferably from 55 to 70° C. The softening temperature is preferably from 90 to 110° C., and more preferably from 90 to 105° C.

The use of a thermoplastic resin falling within the foregoing range of the number-average molecular weight preferably prevents such troubles that when a full-color solid image is bent, an image portion peels, causing image defects (or fixability on bending is deteriorated) and heat-fusibility in fixing is lowered. When a Mw/Mn is within the foregoing range, high temperature off-set hardly occurs, superior sharp melting characteristic results, and light-transmittance of a toner and mixing of color at the time of full color image formation can be prevented. The use of a thermoplastic resin having a

glass transition point falling within the range described above can maintain heat resistance, causes no coagulation of toner particles during storage and can prevent color mixing at the time of forming full color images. The use of a thermoplastic resin falling within the foregoing range of the softening temperature can prevent occurrence of high temperature off-set, maintaining fixing strength, light-transmittance, color mixing and glossiness of full color images at a given level.

There will be now described resin forming the interior (or core) of the colored microparticle of this invention. Resins usable for the interior (core) of the colored microparticle are not specifically limited so long as it differs in composition from the thermoplastic resin described above. Examples thereof include (meth)acrylate resin, polyester resin, polyamide resin, polyimide resin, polystyrene resin, polyepoxy resin, polyester resin, amino type resin, fluorinated resin, phenol resin, polyurethane resin, polyethylene resin, polyvinyl chloride resin, polyvinyl alcohol resin, polyether resin, polyether ketone resin, polyphenylene sulfide resin, polycarbonate resin, and aramid resin. Of these resins, resins obtained by polymerization of ethylenically unsaturated monomers are preferred, such as (meth)acrylate resin, polystyrene resin, polyethylene resin, polyvinyl chloride resin and polyvinyl alcohol resin. (meth)acrylate resin and polystyrene resin are specifically preferred.

(Meth)acrylate resin can be synthesized by homopolymerization or copolymerization of various methacrylate monomers or acrylate monomers and a desired (meth)acrylate resin can be obtained by changing the kind of a monomer or composition ratio of monomers. The (meth)acrylate monomer may be copolymerized with copolymerizable unsaturated monomers other than the (meth)acrylate monomer or may be blended with other resins.

Examples of a monomer forming a (meth)acrylate resin include (meth)acrylic acid, methyl(meth)acrylate, ethyl (meth)acrylate, propyl(meth)acrylate, butyl(meth)acrylate, isopropyl(meth)acrylate, isobutyl(meth)acrylate, t-butyl (meth)acrylate, stearyl(meth)acrylate, 2-hydroxy(meth)acrylate, acetoacetoxyethyl(meth)acrylate, dimethylaminoethyl(meth)acrylate, 2-hydroxypropyl(meth)acrylate, di(ethylene glycol)ethyl ether(meth)acrylate, ethylene glycol methyl ether(meth)acrylate, isobonyl(meth)acrylate, chloroethyltrimethylammonium(meth)acrylate, trifluoroethyl (meth)acrylate, octafluoropentyl(meth)acrylate, 2-acetoamidomethyl(meth)acrylate, 2-methoxyethyl(meth)acrylate, 2-dimethylaminoethyl(meth)acrylate, 3-trimethoxysilanepropyl(meth)acrylate, benzyl(meth)acrylate, tridecyl (meth)acrylate, 4-hydroxybutyl(meth)acrylate, tetrahydrofuryl(meth)acrylate, dodecyl(meth)acrylate, octadecyl(meth)acrylate, 2-diethylaminoethyl(meth)acrylate, 2-ethylhexyl (meth)acrylate, cyclohexyl(meth)acrylate, phenyl(meth)acrylate, and glycidyl(meth)acrylate of these, (meth)acrylic acid, methyl(meth)acrylate, ethyl(meth)acrylate, propyl (meth)acrylatebutyl, butyl(meth)acrylate, stearyl(meth)acrylate, 2-hydroxyethyl(meth)acrylate, acetoacetoxyethyl(meth)acrylate, benzyl(meth)acrylate, tridecyl(meth)acrylate, dodecyl(meth)acrylate, and 2-ethylhexyl(meth)acrylate are preferred.

Polystyrene resins include a styrene homopolymer, and a random copolymer, block copolymer and graft copolymer obtained by copolymerization of a styrene monomer with other copolymerizable unsaturated monomers. A blend of such a styrene polymer and other polymers, or a polymer alloy is also usable.

Examples of a styrene monomer include styrene, an 65 nuclear alkyl-substituted styrene such as  $\alpha$ -methylstyrene,  $\alpha$ -ethylstyrene,  $\alpha$ -methylstyrene-p-methylstyrene, o-meth-

ylstyrene, or p-methylstyrene; and a nuclear halogen-substituted styrene such as o-chlorostyrene, m-chlorostyrene, p-bromoostyrene and tribromostyrene. Of these, styrene or  $\alpha$ -methylstyrene is preferred.

5 The foregoing monomer components are subjected to homopolymerization or copolymerization to obtain resin usable in this invention. Examples thereof include a copolymer resin of a copolymer resin of benzylmethacrylate/ethyl acrylate or butyl acrylate, a copolymer resin of methyl methacrylate/2-ethylhexyl methacrylate, copolymer resin of methyl methacrylate/methacrylic acid/stearyl methacrlate/ 10 acetoacetoxyethyl methacrylate, copolymer resin of styrene/ acetoacetoxyethyl methacrylate/stearyl methacrylate, copolymer resin of styrene/2-hydroxyethyl methacrylate/ 15 stearyl methacrylate, and copolymer resin of 2-ethylhexyl methacrylate/2-hydroxyethyl methacrylate.

The number-average molecular weight of a resin used for the interior (core) is preferably from 500 to 100,000, and more preferably from 1,000 to 30,000 in terms of durability 20 and microparticle-forming ability.

Resin used for a shell, which covers the interior (or core) of the colored microparticle to form a shell, is not specifically limited. Examples thereof include poly(meth)acrylate resin, 25 polyester resin, polyamide resin, polyimides resin, polystyrene resin, polyepoxy resin, amino typeresin, fluorinated resin, phenol resin, polyurethane resin, polyethylene resin, polyvinyl chloride resin, polyvinyl alcohol resin, polyallylate resin, polyether resin polyether ketone resin, polyphenylene sulfide resin, polycarbonate resin and aramid resin. Of these, poly 30 (meth)acrylate resin is preferred in terms of the combination with thermoplastic resin.

(Meth)acrylate resin can be synthesized by homopolymerization or copolymerization of various methacrylate monomers or acrylate monomers and a desired (meth)acrylate resin can be obtained by changing the kind of a monomer or composition ratio of monomers. The (meth)acrylate monomer may be blended with other resins.

Examples of a monomer forming a (meth)acrylate resin include (meth)acrylic acid, methyl(meth)acrylate, ethyl (meth)acrylate, propyl(meth)acrylate, butyl(meth)acrylate, isopropyl(meth)acrylate, isobutyl(meth)acrylate, t-butyl (meth)acrylate, stearyl(meth)acrylate, 2-hydroxy(meth)acrylate, acetoacetoxyethyl(meth)acrylate, dimethylaminoethyl(meth)acrylate, 2-hydroxypropyl(meth)acrylate, di(ethylene glycol)ethyl ether(meth)acrylate, ethylene glycol methyl ether(meth)acrylate, isobonyl(meth)acrylate, chloroethyltrimethylammonium(meth)acrylate, trifluoroethyl (meth)acrylate, octafluoropentyl(meth)acrylate, 2-acetoamidomethyl(meth)acrylate, 2-methoxyethyl(meth)acrylate, 2-dimethylaminoethyl(meth)acrylate, 3-trimethoxysilanepropyl(meth)acrylate, benzyl(meth)acrylate, tridecyl (meth)acrylate, 4-hydroxybutyl(meth)acrylate, tetrahydrofuryl(meth)acrylate, dodecyl(meth)acrylate, octadecyl(meth)acrylate, 2-diethylaminoethyl(meth)acrylate, 2-ethylhexyl (meth)acrylate, cyclohexyl(meth)acrylate, phenyl(meth)acrylate, and glycidyl(meth)acrylate. Of these, (meth)acrylic acid, methyl(meth)acrylate, ethyl(meth)acrylate, propyl (meth)acrylatebutyl, butyl(meth)acrylate, stearyl(meth)acrylate, 2-hydroxyethyl(meth)acrylate, acetoacetoxyethyl(meth)acrylate, benzyl(meth)acrylate, tridecyl(meth)acrylate, dodecyl(meth)acrylate, and 2-ethylhexyl(meth)acrylate are preferred; and methyl(meth)acrylate, ethyl(meth)acrylate, propyl(meth)acrylate and butyl(meth)acrylate are more preferred.

A resin used for the shell may be a copolymer with a reactive emulsifying agent. Reactive emulsifying agents

usable in this invention may be anionic or nonionic ones but compounds containing the following substituent A, B or C:

A: straight chain or branched alkyl, or substituted or unsubstituted aromatic group having at least 6 carbon atoms,

B: nonionic or anionic substituent expressing surface-activity, and

C: radical-polymerizable group.

Example of a straight chain alkyl group described in the foregoing A include heptyl, octyl, nonyl and decyl; example of a branched alkyl group include 2-ethylhexyl; and example of an aromatic group include phenyl, nonylphenyl and naphthyl.

Example of a nonionic substituent expressing surface-activity (emulsifying capability), described in the foregoing B include polyethylene oxide, polypropylene oxide and their copolymer polyalkylene oxide. Example of an anionic substituent include a carboxylic acid, phosphoric acid, sulfonic acid and their salts. An anionic group which substitutes the terminal end of an alkylene oxide, is a specific example of the foregoing anionic substituent. The substituent of the foregoing B is preferably an anionic group, and more preferably one which forms a salt at the terminal end.

The radical-polymerizable group is a group capable of undergoing radical polymerization or a group capable of causing polymerization or cross-linking reaction via a radical active species. Examples thereof include groups containing an ethylenically unsaturated bond, such as a vinyl group, allyl group, isopropenyl group, acryl group, methacryl group, maleimide group, acrylamide group or styryl group.

Preferred emulsifying agents usable in this invention are compounds represented by formula (1) to (3) described below.

Formula (1)



In the foregoing formula (1), R<sub>1</sub> is a straight chain or branched alkyl, or substituted or unsubstituted aromatic group having 6 to 20 carbon atoms group, for example, straight chain alkyl group such as heptyl, octyl, nonyl, decyl or dodecyl, a branched alkyl group such as 2-ethylhexyl, and an aromatic group such as phenyl, nonylphenyl, naphthyl, as described in the foregoing A; R<sub>2</sub> is a radical-polymerizable group, for example, a group containing an ethylenically unsaturated bond, such as acryl group, methacryl group or maleimide group, as described in the foregoing C; Y<sub>1</sub> is a sulfonic acid, carboxylic acid or their salts.

The compound of formula (1) can be synthesized by methods known in the art. It is also commercially available and examples thereof include LATEMUL S-120, LATEMUL S-120A, LATEMUL 180 and LATEMUL S-180A which are all available from Kao Corp.; and ELEMELON JS-2, available from SANYO CHEMICAL INDUSTRIES, LTD.

Formula (2)



In the formula (2), R<sub>3</sub> is the same as defined in R<sub>1</sub> of the foregoing formula (1); R<sub>4</sub> is the same as defined in R<sub>2</sub> of the foregoing formula (1); Y<sub>2</sub> is a sulfonic acid, carboxylic acid or their salts; AO represents an alkylene oxide.

The compound of formula (2) can be synthesized by methods known in the art. It is also commercially available and examples thereof include NE-series of ADEKA REASOAP NE-10, ADEKA REASOAP NE-20 and ADEKA REASOAP NE-30, SE-series of ADEKA REASOAP SE-10N, ADEKA REASOAP SE-20N and ADEKA REASOAP SE-30N, which as all available from ASAHI DENKA KOGYO K.K., RN-series of AQUALON RN-10, AQUALON RN-20, AQUALON RN-30, AQUALON RN-50, HS-series of AQUALON HS-10 and AQUALON HS-20, AQUALON HS-30, and AQUALON BC-series, which are all available from DAIICHI SEIYAKU CO., LTD.



In the formula (3), R<sub>5</sub> is the same as defined in R<sub>1</sub> of the foregoing formula (1); R<sub>6</sub> is the same as defined in R<sub>2</sub> of the foregoing formula (1); Y<sub>2</sub> is the same as defined in Y<sub>1</sub> of the foregoing formula (2).

The compound of formula (3) can be synthesized by methods known in the art. It is also commercially available and examples thereof include KH-series of AQUALON KH-05, AQUALON KH-10, and AQUALON RN-20, which are all available from DAIICHI SEIYAKU CO., LTD.

In the foregoing formulas (2) and (3), the average polymerization degree (n) of an alkylene oxide chain (AO) is preferably from 1 to 10, including, for example, AQUALON KH-05, AQUALON KH-10, AQUALON HS-05, AQUALON HS-10, which are all available from DAIICHI SEIYAKU CO., LTD.

In this invention, anionic reactive emulsifying agents are 35 preferred and examples thereof include ADEKA REASOAP SE-series (available from ASAHI DENKA KOGYO K.K., AQUALON HS-series, available from DAIICHI SEIYAKU CO., LTD., RAMTEL S-series, available from Kao Corp. and ELEMELON JS-series, available from SANYO CHEMICAL INDUSTRIES, LTD.

In this invention, the foregoing reactive emulsifying agents are used preferably in an amount of 0.1 to 80 parts by weight per 100 parts by weight of the total amount of resin forming colored microparticles, more preferably 1 to 70 parts by weight, and still more preferably 10 to 60 parts by weight.

In the process of preparation of colored microparticles relating to this invention, emulsification can be undergone optionally using conventional anionic emulsifying agents (surfactants) and/or nonionic emulsifying agents (surfactants).

Examples of conventional nonionic emulsifying agents include polyoxyethylene alkyl ethers such as polyoxyethylene lauryl ether and polyoxyethylene stearyl ether; polyoxyethylene alkylphenyl ethers such as polyoxyethylene nonylphenyl ether; sorbitan higher fatty acid esters such as sorbitan monolaurate, sorbitan monostearate, and sorbitan trioleate; polyoxyethylene sorbitan higher fatty acid esters, such as polyoxyethylene sorbitan monolaurate; polyoxyethylene higher fatty acid esters such as polyoxyethylene monolaurate and polyoxyethylene monostearate; glycerin higher fatty acid esters such as oleic acid monoglyceride and stearic acid monoglyceride; and polyoxyethylene-polyoxypropylene block copolymer.

Examples of conventional anionic emulsifying agents 65 include higher fatty acid salts such as sodium oleate, alkylarylsulfonates such as sodium dodecylbenzenesulfonate, alkyl sulfonic acid esters such as sodium laurylsulfate, polyoxyeth-

ylene alkyl ether sulfuric acid ester salts such as polyethoxyethylene lauryl ether sulfuric acid sodium salt, polyoxyethylene alkylaryl ether sulfuric acid esters such as polyoxyethylene nonylphenyl ether sulfuric acid sodium salt, alkyl sulfosuccinic acid ester salts such as monoocetyl sulfosuccinic acid sodium salt, dioctyl sulfosuccinic acid sodium salt, and polyoxyethylene laurylsulfosuccinic acid sodium salt, and derivatives of the foregoing.

There will be now described dyes contained in the colored microparticles of this invention. Generally known dyes are usable in this invention, and oil-soluble dyes are preferred and chelate dyes are more preferred.

Usually, oil-soluble dyes which do not contain any water-solubilizing group such as a carboxylic acid or sulfonic acid group, are soluble in organic solvents and not soluble in water, but a dye obtained by salt-formation of a water-soluble dye with a long chain base and thereby being soluble in oil, is also included. There are known, for example, an acid dye, a direct dye and a salt formation dye of a reactive dye with a long chain amine. Specific examples thereof are described below but are not limited to these: Valifast Yellow 4120, Valifast Yellow 3150, Valifast Yellow 3108, Valifast Yellow 2310N, Valifast Yellow 1101, Valifast Red 3320, Valifast Red 3304, Valifast Red 1306, Valifast Blue 2610, Valifast Blue 2606, Valifast Blue 1603, Oil Yellow GG-S, Oil Yellow 3G, Oil Yellow 129, Oil Yellow 107, Oil Yellow 105, Oil Scarlet 308, Oil Red RR, Oil Red OG, Oil Red 5B, Oil Pink 312, Oil Blue BOS, Oil Blue 613, Oil Blue 2N, Oil Black BY, Oil Black BS, Oil Black 860, Oil Black 5970, Oil Black 5906, Oil Black 5905, which are all available from Orient Kagaku Kogyo Co., Ltd.; Kayaset Yellow SF-G, Kayaset Yellow K-CL, Kayaset Yellow GN, Kayaset Yellow A-G, Kayaset Yellow 2G, Kayaset Red SF-4G, Kayaset Red K-BL, Kayaset Red A-BR, Kayaset Magenta 312, Kayaset Blue K-FL, which are all available from NIPPON KAYAKU CO., LTD.; FS Yellow 1015, FS Magenta 1404, FS cyan 1522, FS Blue 1504, C.I. Solvent Yellow 88, 83, 82, 79, 56, 29, 16, 14, 04, 03, 02, and 01; C.I. Solvent Red 84:1, C.I. Solvent Red 84, 218, 132, 73, 72, 51, 43, 27, 24, 18, and 01; Solvent Blue 70, 67, 44, 40, 35, 11, 02, and 01; C.I. Solvent Black 43, 70, 34, 29, 27, 22, 7, 3, and 3; C.I. Solvent Violet 3; C.I. Solvent Green 3 and 7; Plast Yellow DY352, Plast Red 8375, which are available from Arimoto Kagaku Kogyo Co., Ltd.; MS Yellow HD-180, MS Red G, MS Magenta HM-1450H, MS Blue HM-1384, which are available from Mitsui Kagaku Kogyo; ES Red 3001, ES Red 3002, ES Red 3003, TS Red 305, ES Yellow 1001, ES Yellow 1002, Ts Yellow 118, ES Orange 2001, ES Blue 6001, TS Tuyq Blue 618, which are available from SUMITOMO CHEMICAL CO., LTD.; ACROLEX Yellow 6G, Ceres Blue GNNEOPAN Yellow 075, Ceres Blue GN, MACROLEX Red and Violet R, which are available from Bayer Co.

Disperse dyes are also usable as an oil-soluble dye, examples thereof include C.I. Disperse Yellow 5, 42, 54, 64, 79, 82, 83, 93, 99, 100, 119, 122, 124, 126, 160, 184:1, 186, 198, 199, 204, 224 and 237; C.I. Disperse Orange 13, 29, 31:1, 33, 49, 54, 55, 66, 73, 118, 119 and 163; C.I. Disperse Red 54, 60, 72, 73, 86, 88, 91, 92, 93, 111, 126, 127, 134, 135, 143, 145, 152, 153, 154, 159, 164, 167:1, 177, 181, 204, 206, 207, 221, 239, 240, 258, 277, 278, 283, 311, 323, 343, 348, 356 and 362; C.I. Disperse Violet 33; C.I. Disperse Blue 56, 60, 73, 87, 113, 128, 143, 148, 154, 158, 165, 165:1, 165:2, 176, 183, 185, 197, 198, 201, 214, 224, 225, 257, 266, 267, 287, 354, 358, 365 and 368; C.I. Disperse green 6:1 and 9.

In addition, phenol, naphthols; cyclic methylene as pyrazolone and pyrazolotriazole, couplers such as ring-opening

methylene compounds, p-diaminopyridines, azomethine dyes and indoaniline dyes are also usable as an oil-soluble dye.

A metal chelate dye usable in this invention refers to a compound in which a dye coordinates with a metal ion through at least two-dentate coordination and which may contain a ligand other than the dye. The ligand refers to an atomic group capable of coordinating with a metal ion, which may contain a charge or not. Metal chelate dyes usable in this invention are, for example, compounds represented by the following formula (4):



wherein M is a metal ion, "Dye" is a dye capable of coordinating with a metal ion, A is a ligand except for that the Dye, L is 1, 2 or 3, and m is 0, 1, 2 or 3, provided that when m is 0, L is 2 or 3, in which plural "Dye"s may be the same or different. The metal ion represented by M is a metal ion chosen from groups 1 to 9 inclusive of the periodical table of elements, for example, Al, Co, Co, Cr, Cu, Fe, Mn, Mo, Ni, Sn, Ti, Pt, Pd, Zr, and Zn. Ni, Cu, Cr, Co, Zn, and Zn ions are specifically preferred.

Chelate dyes described in JP-A Nos. 9-277693, 10-20559 and 10-30061 are specifically preferred, which is a metal chelate dye formed by allowing at least one dye represented by the following formulas (1) to (6) to be bonded to a metal ion through coordination of the coordination number (or dentate number) of 2 or more:



In the foregoing formulas (1) to (5),  $X_1$  and  $X_2$  are each a group forming a dye through a conjugated system and represent a group or atomic group which is capable of forming a chelate of bi- or more-dentate; Y is an atomic group necessary to form an aromatic carbon ring or a 5- or 6-membered heterocyclic ring. In the formula (6),  $X_3$  is an atomic group capable of linking via a conjugated system;  $Z_1$  and  $Z_2$  are each an atomic group necessary to form a nitrogen-containing heterocyclic ring, in which  $Z_1$  and  $Z_2$  may be the same or

**11**

different. In the formulas (1) to (3) and (6), R<sub>1</sub>, R<sub>2</sub> and R<sub>3</sub> are each a hydrogen atom, a halogen atom or a univalent substituent; and n is 0, 1 or 2.

Specific Examples of such a metal chelate dye usable in this invention are shown below but are by no means limited to these.

**12**

-continued

D-6



-continued



-continued

D-12

5

Ni(OH)<sub>2</sub>

D-13

15

Ni(ClO<sub>4</sub>)<sub>2</sub>

20



D-14

25

NiCl<sub>2</sub>

30



D-15

35

Ni(CH<sub>3</sub>COO)<sup>-</sup><sub>2</sub>

D-16

40

Ni(CH<sub>3</sub>COO)<sup>-</sup><sub>2</sub>

45



D-17

50

Ni(C<sub>6</sub>H<sub>5</sub>COO)<sup>-</sup><sub>2</sub>

55



D-18

60

Ni(C<sub>6</sub>H<sub>5</sub>COO)<sup>-</sup><sub>2</sub>

65



D-18

D-19

D-20

D-21

D-22

Ni<sup>2+</sup>

D-23

Ni<sup>2+</sup>

**15**

-continued



D-35

5  
10  
D-3615  
20  
D-3725  
30  
D-3835  
D-3940  
45  
D-4050  
55  
60  
65

-continued



D-41



D-42



D-43



D-44



D-45

CoCl<sub>2</sub>

**19****20**

-continued

D-47

 $\text{Ni}^{2+}(\text{C}_2\text{H}_5\text{COO}^-)_2$ 

5



D-53

 $\text{Ni}(\text{OH})_2$ 

D-48

 $\text{Ni}^{2+}$ 20  
25

D-54

 $\text{Zn}^{2+}(\text{CH}_3\text{COO}^-)_2$ NH<sub>2</sub>  
30  
35

D-55

 $\text{Ni}(\text{OH})_2$ D-50  
40  
45 $\text{NiCl}_2$ 

D-56

 $\text{Ni}(\text{ClO}_4)_2$ D-51  
50 $\text{Ni}(\text{ClO}_4)_2$  $\text{Ni}^{2+}$ 

D-59

 $\text{Ni}^{2+}$ 

D-52

 $\text{NiCl}_2$ 60  
65 $\text{Ni}(\text{BF}_4)_2$

-continued



-continued

D-67



23

24



25



26



27





are-useable salicylic acid metal complexes described, for example, in JP-A Nos. 53-127726 and 62-145255; carixarene compounds described, for example, in JP-A No. 2-201378; organic borane compounds described, for example, in JP-A Nos. 2-221967 and 3-1162. Such a charge control agent is used preferably in an amount of 0.1 to 10 parts by weight per 100 parts by weight of thermoplastic resin (binding resin), and more preferably 0.5 to 5.0 parts by weight.

Off-set preventing agents usable in this invention are not specifically limited and specific examples thereof include polyethylene wax, oxidation type polyethylene wax, polypropylene wax, oxidation type polypropylene wax, carnauba wax, sazole wax, rice wax, candelilla wax, jojoba wax, and bees wax. Such a wax is used preferably in an amount of 0.5 to 5.0 parts by weight per 100 parts by weight of thermoplastic resin, and more preferably 1.0 to 3.0 parts by weight. Incorporation of an off-set preventing agent within the foregoing range displays its effects, resulting in superior light-transmittance and color reproduction.

Using a thermoplastic resin, colored microparticles and other desired additives, the toner of this invention can be manufactured by commonly known methods such as a kneading and grinding method, suspension polymerization method, emulsion polymerization method, emulsion granulation method, or capsulation method. Of the foregoing methods, taking into account the decrease of the toner particle size along with enhancement of image quality, the emulsion polymerization method is preferable in terms of manufacturing cost and manufacturing stability.

A thermoplastic resin emulsion prepared by emulsion polymerization is mixed with a dispersion of toner particle components such as colored microparticles. While maintaining balance between repulsion force of the particle surface, formed by pH adjustment and aggregation force due to addition of an electrolyte, aggregation is gradually performed. Association is performed with controlling the particle size and the particle size distribution, while stirring with heating. Thereby, fusion of microparticles and particle shape control are conducted to manufacture the toner particles.

The volume-average particle size of the toner relating to this invention is preferably 4-10  $\mu\text{m}$  in terms of high precise image reproduction, and more preferably 6 to 9  $\mu\text{m}$ . The volume-average particle size can be determined by Coulter Counter TA-II (produced by Coulter Corp.).

In this invention, the thus prepared toner particles may be used as it is, but preferably, external additives may be incorporated to the toner particles to control electrostatic charge or enhance fluidity or cleaning ability. Examples of such external additives include inorganic oxide particles such as particulate silica, particulate alumina, and particulate titania, inorganic stearate compound particles such particulate aluminum stearate or particulate zinc stearate, and inorganic titanate compound particles such as strontium titanate or zinc titanate. These additives may be used singly or in combination. These particles are desirably used together with a surface treatment of a silane coupling agent, titan coupling agent, higher fatty acid or silicone oil in terms of environmental resistance stability and heat resistance maintenance. The external additive is incorporated preferably in an amount of 0.05 to 5 parts by weight per 100 parts by weight of toner particles, and more preferably from 0.1 to 3 parts by weight.

The toner of this invention may be mixed with a carrier and used as a toner used for a two-component developer, or may be used as a toner used for a single-component developer.

Conventional carriers used for a two-component developer can be used in combination with the toner of this invention. There can be used, for example, a carrier composed of mag-

The volume-average particle size of the colored microparticles relating to this invention is preferably 10 nm to 1  $\mu\text{m}$ , and more preferably 20 to 500 nm. A volume-average particle size falling within the foregoing range effects inclusion of a dye into resin of the colored microparticle, easily maintaining standing stability of colored microparticles and leading to superior storage stability. Further, in the process of preparation of colored microparticles, sedimentation is prevented and standing stability is also maintained. When used as a toner, glossiness or transparency is achieved.

The volume-average particle size can be determined by the dynamic light scattering method, laser diffraction method, centrifugal sedimentation method, FFF method or electric detector method. In this invention determination in the dynamic light scattering method using "Zeta Sizer" (produced by Marbahn CO.) is preferable.

The dye content of the colored microparticle is preferably from 10% to 70% by weight, based on the microparticle. A dye content falling within the foregoing range can obtain a sufficient image density, expresses protective capability for the dye and exhibits superior storage stability as a microparticle dispersion, thereby preventing an increase of the particle size due to aggregation.

In addition to the foregoing thermoplastic resin and colored microparticles, a charge control agent or a off-set preventing agent known in the art may be incorporated to the toner of this invention.

Charge control agents usable in this invention are not specifically limited. As a negative charge control agent used for color toners are usable colorless, white or light color charge control agents. Preferred example thereof include zinc or chromium metal complex of salicylic acid derivatives, carixarene compounds, organic borane compounds, and fluorine-containing quaternary ammonium salt compounds. There

31

netic material particles such as iron or ferrite, a resin-coated carrier formed by covering magnetic material particles with resin and a binder type carrier obtained by dispersing powdery magnetic material in a binder. Of these carriers, the use of a resin-coated carrier using silicone resin, copolymer resin (graft resin) of an organopolysioxane and a vinyl monomer or polyester resin is preferred from the viewpoint of toner spent and the like. Specifically, a carrier coated with a resin which is obtained by reacting isocyanate with a copolymer resin of an organopolysiloxane and a vinyl monomer, is preferred in terms of fastness, ecological concerns and resistance to spent toner. A monomer containing a substituent such as a hydroxyl group having reactivity with an isocyanate needs to be used as the above-described vinyl monomer. The volume-average particle size of a carrier is preferably 15 to 100  $\mu\text{m}$  to maintain high image quality and prevent a carrier from fogging. The volume-average particle size of the carrier can be determined using a laser diffraction type particle size distribution measurement apparatus, HELOS (produced by SYMPATEC Corp.).

Next, there will be described an image formation method using the toner of this invention.

In this invention, the system of image formation is not specifically limited. Examples thereof include a system in which plural images are formed on a photoreceptor and transferred all together, a system in which an image formed on a photoreceptor is successively transferred using a transfer belt and is not specifically limited to such, of which the system in which plural images are formed on a photoreceptor and transferred all together is preferred.

In this system, the photoreceptor is uniformly charged and exposed according to the first image and the first development is performed to form the first toner image on the photoreceptor. Subsequently, the photoreceptor having formed the first toner image is uniformly charged, exposed according to the second image and the second development is performed to the second toner image. Further, the photoreceptor having formed the first and second toner images is uniformly charged, exposed according to the third image and the third development is performed to form the third toner image on the photoreceptor. Furthermore, the photoreceptor having formed the first, second and third toner images is uniformly charged, exposed according to the fourth image and the fourth development is performed to form the fourth toner image on the photoreceptor. In the foregoing, the first development is performed with a yellow toner, the second development is performed with a magenta toner, the third development is performed with a cyan toner and the fourth development is performed with a black toner to form a full color image. Thereafter, images formed on the photoreceptor are transferred all together to a transfer material such as paper and fixed on the transfer material to form images. In this system, images formed on the photoreceptor are transferred all together to paper or the like to form the final image, so that differing from a so-called intermediate system, the transfer, which often perturbs the previous images, is done only one time, resulting in enhanced image quality.

Since a plural number of development processes need to be performed to develop latent images formed on the photoreceptor, a non-contact development system is preferred. A

32

system in which an alternant electric field is applied during development, is also preferable.

Suitable fixing systems usable in this invention include a so-called contact heating system. Representative examples of the contact heating system include a heat roll fixing system and a pressure heat-fixing system in which fixing is performed using a rolling pressure member including a fixed heating body.

In the image formation process to perform development, transfer and fixing by using a toner of this invention, the toner transferred onto a transfer material, e.g., paper, adheres onto the paper surface without colored microparticles being disintegrated, even after fixing.

In conventional toners obtained by directly dispersing or dissolving a dye in a thermoplastic resin (binding resin), the dye bleeds out onto the toner particle surface, producing the following problems: (1) low charging, (2) marked difference in charging between high temperature and high humidity, and low temperature and low humidity, (3) the charging amount varying depending on the kind of dye as a colorant, for example, when using pigments of cyan, magenta, yellow and black in full color recording. However, in this invention, colored microparticles are dispersed within the toner particle so that in spite of the toner particle having the dye at a relatively high content, the dye does not bleed out on the particle surface, overcoming the foregoing problems.

Further, when thermally fixed onto a transfer material, transport of a dye as colorant to the outside of the colored microparticles (bleeding-out onto the surface of the colored microparticle) does not result and does not produce problems sublimation of a dye or oil staining during thermal fixing, as tends to be caused with conventional toners.

## EXAMPLES

The present invention will be further described based on examples, but are by no means limited to these.

### Colored Microparticle

#### Preparation of Dispersion of Colored Microparticle 1

To a separable flask were added 13.5 g of resin (P-1), 16.3 g of dye (A-1) and 123.5 g of acetic acid and after the atmosphere in interior was replaced with nitrogen gas, the dye was completely dissolved with stirring. Further thereto, 238 g of an aqueous solution 8.0 g of AQUALON KH-50 (produced by DAIICHI SEIYAKU CO., LTD.) was dropwise added with stirring and then emulsified for 300 sec. using CLEAR-MIX W-MOTION CLM-0.8W (produced by M-TECHNIQUE Co.). Thereafter, acetic acid was removed under reduced pressure to obtain a dispersion of colored microparticles 1 containing a dye. In the thus obtained dispersion, the volume-average particle size of colored particles was 30 nm. Hereinafter, the volume-average particle size was determined using ZETASIZER (Marbahn Co.).

Resin (P-1): St/AAEM/SMA=50/30/20

ST: styrene

AAEM: acetoacetoxyethyl methacrylate

SMA: stearyl methacrylate



Dye (A-1)

## Preparation of Dispersion of Colored Microparticle 2

A dispersion of colored microparticle 2 was prepared similarly to the foregoing dispersion of colored microparticle 1, provided that, further to the dispersion of colored microparticle 1, 0.5 g of potassium persulfate was added and heated at 70°C. using a heated and 10.0 g of methyl methacrylate was dropwise added and allowed to react for 5 hr. The thus obtained dispersion of colored particle 2 was core/shell type colored particles having a shell resin (shell) layer formed on the surface of the colored particle 1 as a core. In the thus obtained dispersion, the volume-average particle size of colored particles was 33 nm.

## Preparation of Dispersion of Colored Microparticle 3

A dispersion of core/shell type colored microparticle 3 was prepared similarly to the foregoing dispersion of colored microparticle 2, provided that the resin (P-1) and dye (A-1) were replaced by resin (P-2) and dye (A-2), respectively. In the thus obtained dispersion, the volume-average particle size of colored particles was 45 nm.

Resin (P-2: St/HEMA/SMA=30/40/30

HEMA: 2-hydroxyethyl methacrylate



## Preparation of Dispersion of Colored Microparticle 5

A dispersion of core/shell type colored microparticle 5 was prepared similarly to the foregoing dispersion of colored microparticle 2, provided that the amount of AQUALON KH-50 was changed varied from 8.0 g to 1.0 g. In the thus obtained dispersion, the volume-average particle size of colored particles was 120 nm.

## Preparation of Dispersion of Colored Microparticle 6

A dispersion of core/shell type colored microparticle 6 was prepared similarly to the foregoing dispersion of colored microparticle 2, provided that the amount of dye (A-1) was changed varied from 16.0 g to 1.0 g. In the thus obtained dispersion, the volume-average particle size of colored particles was 28 nm.

## Preparation of Dispersion of Colored Microparticle 4

A dispersion of core/shell type colored microparticle 4 was prepared similarly to the foregoing dispersion of colored microparticle 2, provided that the resin (P-1) and dye (A-1) were replaced by resin (P-2) and dye (A-3), respectively and methyl methacrylate was replaced by acrylonitrile. In the thus obtained dispersion, the volume-average particle size of colored particles was 70 nm.

Dye (A-2)



## Preparation of Dispersion of Colored Microparticle 7

A dispersion of core/shell type colored microparticle 7 was prepared similarly to the foregoing dispersion of colored microparticle 2, provided that the amount of dye (A-1) was changed varied from 16.0 g to 40.0 g. In the thus obtained dispersion, the volume-average particle size of colored particles was 198 nm.

35

## Preparation of Dispersion of Colored Microparticle 8

A dispersion of core/shell type colored microparticle **8** was prepared similarly to the foregoing dispersion of colored microparticle **2**, provided that the resin (P-1) and dye (A-1) were replaced by resin (P-3), and dye (A-4), respectively. In the thus obtained dispersion, the volume-average particle size of colored particles was 51 nm.

Resin (P-3): ST/HEMA/SMA=20/40/40

ST: styrene

HEMA: 2-hydroxyethyl methacrylate

SMA: stearyl methacrylate



In Table 1 are shown the kind of core resin, shell resin or dye used in the foregoing colored microparticles and the volume-average particle size of the colored microparticles.

TABLE 1

| Colored Microparticle No. | Core Resin | Shell Resin | Dye | Volume-average Particle Size (nm) |
|---------------------------|------------|-------------|-----|-----------------------------------|
| 1                         | P-1        | —           | A-1 | 30                                |
| 2                         | P-1        | MMA         | A-1 | 33                                |
| 3                         | P-2        | MMA         | A-2 | 45                                |
| 4                         | P-2        | AN          | A-3 | 70                                |
| 5                         | P-1        | MMA         | A-1 | 1200                              |
| 6                         | P-1        | MMA         | A-1 | 28                                |
| 7                         | P-1        | MMA         | A-1 | 198                               |
| 8                         | P-3        | MMA         | A-4 | 51                                |

MMA: methyl methacrylate  
AN: acrylonitrile

Toner

## Preparation of Thermoplastic Resin (Latex)

Into 5,000 ml separable flask fitted with a stirring device, a temperature sensor, a condenser and a nitrogen-introducing was charged an aqueous surfactant solution (aqueous medium) of 7.08 g of an anionic surfactant (sodium dodecylbenzenesulfonate) which was previously dissolved in 2760 g of deionized water and the internal temperature was increased with stirring at a stirring rate of 230 rpm under a stream of nitrogen. Separately, 72.0 g of a compound of the following Formula (1) as releasing agent was added to a monomer

36

mixture of 115.2 g of styrene, 42.0 g of n-butyl acrylate and 10.9 g of methacrylic acid and dissolved with heating at 80° C. to prepare a monomer solution. Using a mechanical disperser having a circulation path, the monomer solution (80° C.) was mixed with the foregoing aqueous surfactant solution (80° C.) and stirred to prepare a dispersion of emulsion particles (oil droplets) having a uniform dispersion particle size. Subsequently, to this dispersion, a polymerization initiator solution of 0.84 g of a polymerization initiator (potassium persulfate, KPS) dissolved in 200 g of deionized water was added and heated at 80° C. for 3 hr. with stirring to perform polymerization (first polymerization) to form a latex. Then, to this latex, a polymerization solution of 7.73 g of a polymerization initiator (KPS) dissolved in 240 g of deionized water was added. After 15 min, a monomer mixture of 383.6 g of styrene, 140.0 g of n-butyl acrylate, 36.4 g of methacrylic acid and 13.7 g of tert-dodecylmercaptan was added dropwise at 80° C. over a period of 126 min. After completing addition, stirring continued for 60 min. with heating to perform polymerization (second polymerization). Then the reaction mixture was cooled to 40° C. to obtain a latex. The thus obtained latex was designated as latex (1).



## Preparation of Toner Particle

35 Into 5 lit. separable flask fitted with a stirring device, a temperature sensor, a condenser and a nitrogen-introducing was charged 1250 g of the latex (1), 2,000 ml of deionized water and the dispersion of colored microparticle 1. After adjusting the interior temperature to 30° C., the reaction mixture was adjusted to a pH 10.0 by adding a 5N aqueous sodium hydroxide solution. Then, an aqueous solution of 52.6 g of 40 magnesium chloride hexahydrate which was previously dissolved in 72 ml of deionized water, was added at 30° C. in 10 min. After allowed to stand for 3 min., heating was started and the reaction system was heated to 90° C. in 6 min. (at a temperature-increasing rate of 10° C./min). From that state, 45 measurement of the aggregated particle size was started using Coulter Counter TA-II (produced by Coulter Corp.). When the volume-average particle size reached 6.5 μm, an aqueous solution of sodium chloride of 115 g dissolved in 700 ml of deionized water to stop grain growth and the reaction mixture 50 was further stirred for 6 hr. with maintaining the temperature at 90±2° C. to continue fusion. Thereafter, the reaction mixture was cooled to 30° C. at a rate of 6° C./min. The aggregated particles were filtered off from dispersion of the aggregated particles and dispersed in deionized water in an amount 55 of 10 times the weight of aggregated particles to perform washing. After repeating the procedure of washing and filtration twice, washing was done with deionized water and drying was done by hot air at 40° C. to obtain toner particles. The thus obtained toner particles were designated "toner particle 1".

## Preparation of Toner Particle 2

60 Toner particles were prepared similarly to the foregoing toner particle 1, except that the dispersion of colored microparticle 1 was replaced by the dispersion of colored microparticle 2. The thus obtained toner particles were designated "toner particle 2".

## Preparation of Toner Particle 3

Toner particles were prepared similarly to the foregoing toner particle 1, except that the dispersion of colored micro-particle 1 was replaced by the dispersion of colored micro-particle 3. The thus obtained toner particles were designated "toner particle 3".

## Preparation of Toner Particle 4

Toner particles were prepared similarly to the foregoing toner particle 1, except that the dispersion of colored micro-particle 1 was replaced by the dispersion of colored micro-particle 4. The thus obtained toner particles were designated "toner particle 4".

## Preparation of Toner Particle 5

Toner particles were prepared similarly to the foregoing toner particle 1, except that the dispersion of colored micro-particle 1 was replaced by the dispersion of colored micro-particle 5. The thus obtained toner particles were designated "toner particle 5".

## Preparation of Toner Particle 6

Toner particles were prepared similarly to the foregoing toner particle 1, except that the dispersion of colored micro-particle 1 was replaced by the dispersion of colored micro-particle 6. The thus obtained toner particles were designated "toner particle 6".

## Preparation of Toner Particle 7

Toner particles were prepared similarly to the foregoing toner particle 1, except that the dispersion of colored micro-particle 1 was replaced by the dispersion of colored micro-particle 7. The thus obtained toner particles were designated "toner particle 7".

## Preparation of Toner Particle 8

Toner particles were prepared similarly to the foregoing toner particle 1, except that the dispersion of colored micro-particle 1 was replaced by the dispersion of colored micro-particle 8. The thus obtained toner particles were designated "toner particle 8".

## Preparation of Toner Particle 9

Using a surfactant, a low molecular weight polypropylene (number-average molecular weight of 3200) was dispersed in water at a solid content of 30% by weight to prepare an emulsion of low molecular weight polypropylene. To 60 g of the thus prepared low molecular weight polypropylene emulsion was added 338 g of the dispersion of colored micro-particle 1. Further thereto, 220 g of styrene monomer, 40 g of n-butyl acrylate monomer, 12 g of methacrylic acid monomer, 5.4 g of t-dodecylmercaptan as a chain-transfer and 2,000 ml of degassed water were added, and maintained at 70° C. for 3 hr. with stirring under a stream of nitrogen to perform emulsion polymerization.

The thus obtained particular resin dispersion was adjusted to a pH of 7.0 with sodium hydroxide. Then, 700 ml of an aqueous 2.7 mol % potassium chloride solution was added thereto 420 ml of isopropyl alcohol and 23.4 g of polyoxyethylene octylphenyl ether (ethylene oxide average polymerization degree of 10), which was previously dissolved in 175 ml of pure water and maintained for 6 hr. at 75° C. with stirring to perform reaction. Thereafter, the reaction mixture was cooled to 30° C. at a rate of 6° C./min. The aggregated particles were filtered off from dispersion of the aggregated particles and dispersed in deionized water in an amount of 10 times the weight of aggregated particles to perform washing. After repeating the procedure of washing and filtration twice, washing was done with deionized water and drying was done by hot air at 40° C. to obtain toner particles. The thus obtained toner particles were designated "toner particle 9".

by hot air at 40° C. to obtain toner particles. The thus obtained toner particles were designated "toner particle 9".

## Preparation of Toner Particle 10

To an aqueous solution of sodium dodecylsulfate dissolved in 200 ml of pure water, 20 g of dye (A-1) was added, stirred and dispersed by ultrasonic to prepare a colored particle dispersion. Using a surfactant, a low molecular weight polypropylene (number-average molecular weight of 3200) was dispersed in water at a solid content of 30% by weight to prepare an emulsion of low molecular weight polypropylene. To 60 g of the thus prepared low molecular weight polypropylene emulsion was added 338 g of the dispersion of colored micro-particle 1. Further thereto, 220 g of styrene monomer, 40 g of n-butyl acrylate monomer, 12 g of methacrylic acid monomer, 5.4 g of t-dodecylmercaptan as a chain-transfer and 2,000 ml of degassed water were added, and maintained at 70° C. for 3 hr. with stirring under a stream of nitrogen to perform emulsion polymerization.

The thus obtained particular resin dispersion was adjusted to a pH of 7.0 with sodium hydroxide. Then, 675 ml of an aqueous 2.7 mol% potassium chloride solution was added thereto 400 ml of isopropyl alcohol and 22.5 g of polyoxyethylene octylphenyl ether (ethylene oxide average polymerization degree of 10), which was previously dissolved in 168 ml of pure water and maintained for 6 hr. at 75° C. with stirring to perform reaction. Thereafter, the reaction mixture was cooled to 30° C. at a rate of 6° C./min. The aggregated particles were filtered off from dispersion of the aggregated particles and dispersed in deionized water in an amount of 10 times the weight of aggregated particles to perform washing. After repeating the procedure of washing and filtration twice, washing was done with deionized water and drying was done by hot air at 40° C. to obtain toner particles. The thus obtained toner particles were designated "toner particle 10".

## Preparation of Toner Particle 11

Toner particles were prepared similarly to the foregoing toner particle 9, except that the dye (A-1) was replaced by C.I. Pigment Blue 15-3 (produced by Dainippon Ink Kagaku Kogyo). The thus obtained toner particles were designated "toner particle 11".

To each of the toner particle 1 to 11, hydrophobic silica (having a number-average particle size of 12 nm and a hydrophobicity degree of 68) and hydrophobic titanium (having a number-average particle size of 20 nm and a hydrophobicity degree of 63) as external additives were added at 1% by weight and 1.2% by weight, respectively and mixed for 15 min. using a Henschel mixer (produced by Mitsui Miike Kako-sha). Thereafter, coarse particles were removed using a sieve having an opening of 45 µm to obtain Toners 1 to 11. These were also denoted "Inv. 1 to 9" and "Comp. 1 and 2".

## Preparation of Developer

A silicone resin-covered ferrite carrier having a volume-average particle size of 60 µm was mixed with each of the foregoing toners 1 to 11 at a toner content of 6% by weight to obtain "developer 1" to "Developer 11".

## Evaluation

Digital copier Konica 7075 (produced by Konica Minolta Business Technology, Inc.) was used as an apparatus for evaluation, in which a fixing device was modified as below.

A heat-roll fixing system was used as a fixing device. Thus, a heating roller was formed by covering the core surface of an aluminum alloy cylinder (having an inside diameter of 40

mm, a thickness of 1.0 mm and a total width of 310 mm) including a heater in the central portion, using a 120  $\mu\text{m}$  thick tube of copolymer of tetrafluoroethylene and perfluoroalkyl vinyl ether (PFA). A pressure roller was formed by covering the core surface of an iron cylinder (having an inside diameter of 40 mm and a thickness of 2.0 mm), using a sponge-form silicone rubber (having an ASKER C hardness of 48 and a thickness of 2 mm). The heating roller was brought into contact with the pressure roller to form a 5.5 mm wide nip. Using this fixing apparatus, the print speed was set to 480 mm/sec. A supply system in which a web system was impregnated with polydiphenylsilicone (exhibiting a viscosity of 10 Pa·s at 20° C.), was employed as a cleaning mechanism of the fixing device. The fixing temperature was controlled based on the surface temperature of the heating roller (setting temperature: 175° C.). The coating amount of silicone oil was 0.1 mg/A4.

Evaluation was made under an environment of ordinary temperature and ordinary humidity (25° C., 55% RH) and the development conditions were set as follows:

Photoreceptor surface potential: -700 V

DC bias: -500 V

D<sub>sd</sub> (distance between photoreceptor and development sleeve): 600  $\mu\text{m}$

Developer layer control: magnet type (H-Cut system)

Developer layer thickness: 700  $\mu\text{m}$

Development sleeve: 40 mm.

Using the toners obtained above in the apparatus for evaluation under the foregoing evaluation conditions, practical picture tests were done on fine-quality paper and an OHP sheet, and evaluation was made with respect to (1) color reproduction, (2) transparency, (3) charging property, (4) off-set resistance and (5) heat resistance of the respective toners.

#### (1) Color Reproduction

Color reproduction of monochrome images was visually evaluated by ten persons based on the following criteria. Evaluation was conducted in a toner-deposit amount of  $0.7 \pm 0.05 \text{ mg/cm}^2$ .

A: excellent color reproduction,

B: superior color reproduction,

C: slight color staining but acceptable in practice,

D: marked color staining and unacceptable in practice.

#### (2) Transparency

A transparent image formed on an OHP sheet was prepared and the fixed image was measured with respect to visible spectral absorbance by Type 330 Spectrophotometer (produced by HITACHI) using an OHP sheet having no toner as a reference. There were determined the difference in absorbance between 650 nm and 450 nm of a yellow toner, the difference in absorbance between 650 nm and 550 nm of a magenta toner, and the difference in absorbance between 500 nm and 600 nm of a cyan toner. Transparency of the individual OHP image was evaluated based on the following criteria, in which a value of at least 70% was judged to be good transparency. Evaluation was conducted in a toner deposit amount of  $0.7 \pm 0.05 \text{ mg/cm}^2$ .

A: 90% or more, being superior,

B: 70%-90%, being good

C: less than 70%, being no good.

#### (3) Charging Property

Evaluation of charging property was conducted by varying the electrostatic charge of every print. Thus, based on the following criteria, the value of  $Q_b/Q_a$  was evaluated, where  $Q_a$  is the electrostatic charge after setting a developer and

making the first print and  $Q_b$  is the electrostatic charge after completion of printing of 1,000,000 sheets.

A: not less than 0.9 and less than 1.1, being superior,

B: not less than 0.8 and less than 0.9, or not less than 1.1 and less than 1.2, being good,

C: not less than 0.7 and less than 0.8, or not less than 1.2 and less than 1.3, being acceptable in practice,

D: less than 0.7 or more than 1.3, being unacceptable in practice.

#### (4) Off-Set Resistance

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545

**41**

3. The toner of claim 1, wherein the dye is a metal chelate dye.
4. The toner of claim 1, wherein the colored microparticles have a volume-average particle size of 10 nm to 1  $\mu\text{m}$ .
5. The toner of claim 2, wherein the resin (2) is a (meth) acrylate resin.
6. The toner of claim 1, wherein the dye content of the colored microparticles is 10% to 70% by weight.

5

**42**

7. An image forming method comprising: imagewise exposing a uniformly charged photoreceptor to form an electrostatic latent image, developing the electrostatic latent image with a toner to form a toner image and transfer the toner image to a transfer material, wherein the toner is a toner as claimed in claim 1.

\* \* \* \* \*